

2,851,417

## COMPLEX ALKOXY METAL SALTS OF ORGANIC ACIDS AND LUBRICATING AND FUEL COMPOSITIONS THEREOF

Harry J. Andress, Jr., Pitman, N. J., assignor to Secony Mobil Oil Company, Inc., a corporation of New York

No Drawing. Application April 10, 1953  
Serial No. 348,117

9 Claims. (Cl. 252—33)

This invention relates to improved petroleum fractions, such as gasolines, fuels and lubricating oils. More particularly, it relates to a new class of multi-functional additives for such fractions and to a method for their preparation.

It is well known that substantially all mineral oil fractions refined for their various uses are susceptible to oxidation. The manner in which this oxidation manifests itself varies with the particular oil fraction, the manner of its refinement and the conditions under which it is stored or used. Thus, mineral lubricating oils are subject to oxidative deterioration, particularly under conditions of high temperature and pressure encountered in use in internal combustion engines. This oxidation produces acidic bodies in the oil which are corrosive to the metal parts of the engine, particularly to certain types of alloys, such as copper-lead and cadmium-silver alloys, utilized in present day engines. This oxidative deterioration is also attended by deposition of carbonaceous sludge, lacquer and resinous materials which accumulate in the engine, particularly around the piston ring skirts and grooves, so that the operating efficiency of the engine is impaired.

Another problem encountered with gasolines and fuel oils in pipe lines and in storage is the rusting of the pipe line and container walls, the fuel oil or gasoline thereby being contaminated with rust which produces an undesirable sediment therein. Oxidation in storage also causes color degradation and sediment formation in the gasoline or fuel oil. This rust and oxidation sediment causes plugging of filter screens, orifices, etc. in engines or heating units in which the gasoline or fuel oil is used.

In order to overcome, insofar as possible, the various deleterious effects of oxidation in mineral oil fractions, it has become the practice in the art to add to said fractions minor amounts of chemical agents, which have the ability to minimize these effects. Thus, agents are known which, when added to lubricating oils, are capable of inhibiting to a significant degree the corrosive effect of oxidation on the metal parts of engines. These agents are known as anti-oxidants. Agents are also known which have the ability to keep sedimentation and deposit-forming materials formed in fuel in storage or in a lubricating oil in use in suspension, thereby helping to keep the fuel burning equipment or the engine being lubricated clean and in good operating condition for extended periods of time. Such additives are known as detergents or dispersants. Still other agents are known which act to inhibit other deleterious effects in oil fractions, such as anti-rust agents for gasoline and fuel oils. Ordinarily, a combination of such chemical agents must be utilized in a fuel or a lubricating oil in order to provide all the desired improving effects. The present invention, however, provides a new class of metal organic addition agents which are multi-functional in their activity, i. e., they are capable of improving mineral oil fractions in several respects. Thus, the additives of the invention, which may be designated

as complex metal alkoxy salts of organic acids, are excellent detergents as well as highly effective anti-oxidants for lubricating oils. Furthermore, they act as stabilizers for fuel oils in that they prevent color degradation and sedimentation therein. Finally, these complex salts are excellent anti-rust and anti-screen clogging agents for gasolines and fuel oils.

As far as is known, the complex salts herein contemplated have not been prepared heretofore and they are, therefore, considered to be new compositions of matter.

It is, therefore, an object of this invention to provide a new class of complex alkoxy metal salts. It is a further object to provide lubricating oil compositions containing relatively small amounts of these new complex alkoxy metal salts, which compositions are improved with respect to their anti-corrosive and detergents properties. It is also an object to provide gasoline and fuel oil compositions containing minor amounts of these salts whereby such compositions are improved in their anti-oxidant, anti-screen clogging and anti-rust properties. Other and further objects will become apparent from the following detailed description of the invention.

Broadly stated, the complex alkoxy salts of the invention are high metal content complex salts prepared by the reaction of an oil-soluble organic acid with a metal alcoholate in a proportion such as to supply to the reaction an excess of metal alcoholate over that which would be equivalent to the acid-hydrogen content of the organic acid.

The complex alkoxy metal salts thus provided by the invention contain at least about 2 and up to about 6 equivalents of metal. The reaction is conducted by heating together a solvent solution of the organic acid and an alcohol solution of the metal alcoholate reactant for several hours. Temperatures suitable for the reaction range, broadly, from about 50° C. up to about 200° C., the particular temperature utilized in any case being that sufficient to effect the removal of the alcohol from the reaction mixture by distillation, in the course of the reaction, but not high enough to remove the solvent, which is generally a hydrocarbon solution, preferably a mineral lubricating oil. In this way, a fluid concentrate of the complex metal alcoholate salt is obtained, which is readily filtered to remove insolubles and which is adaptable for addition to the particular oil fraction which it is desired to improve. Hydrocarbon solvents other than mineral lubricating oil may, of course, be utilized, such as light naphtha, kerosene, toluene, xylene or the like. These may or may not be removed from the complex salt product prior to addition to a petroleum fraction.

As aforesaid, from 2 and up to 6 equivalents of metal may be incorporated into the complex methoxy salt product depending upon the amount of metal alcoholate reactant used. From 2 to about 6 equivalents of metal alcoholate, based on the equivalents of acid-hydrogen in the organic acid, are, therefore, ordinarily used in the reaction. A general procedure for conducting the reaction is as follows: The organic acid reactant is dissolved in mineral lubricating oil. A slurry of the metal alcoholate reactant, in alcohol, is then prepared. This slurry is then added to the oil solution of the organic acid with constant stirring to form an intimate mixture of the reactants. When the addition is complete, the reaction mixture is heated with stirring to a temperature of, say, from about 120° C. to about 175° C. for from about one hour to about six hours in order to complete the reaction. Any excess alcohol remaining in the reaction mixture is then removed by further heating at a higher temperature and/or reduced pressure. The product, which is an oil solution of the complex alkoxy metal salt, is then filtered to remove any traces of insolubles.

The aforescribed procedure may, of course, be varied without affecting the reaction or the yield of complex salt product obtained. Thus, the manner of bringing the reactants together is not of material significance, it being only necessary that a good mixture of the reactants be obtained.

Due to the complex nature of the alkoxy metal salt products of the invention, it has not been possible to determine their exact chemical structure and they are, therefore, defined and claimed herein in terms of their method of preparation.

#### THE ORGANIC ACID REACTANT

As far as is known, all organic acids will react with the metal alcoholates in accordance with the invention to form high metal content complex salts of the type herein contemplated. The acids particularly contemplated herein, however, are the oil-soluble organic acids. These have relatively high molecular weights, i.e., about 200 or above. Those acids having molecular weights of from about 300 to about 1000 are particularly preferred. More specifically, the following types of acids are particularly contemplated herein.

(a) Carboxylic acids of the aliphatic, aromatic or naphthenic type, the aliphatic acids having at least about 10 and up to about 24 carbon atoms and the aromatic acids and naphthenic acids having aliphatic substituent groups containing at least about 10 and up to about 24 carbon atoms. As non-limiting examples of such acids, there may be mentioned aliphatic carboxylic acids such as decanoic acid, lauric acid, stearic acid, oleic acid, linoleic acid, arachidic acid, abietic acid, etc.; aromatic carboxylic acids, such as alkyl-substituted benzoic, salicylic and phthalic acids, where the alkyl group or groups are attached to the aryl nucleus of the acid and contain a total of at least about 10 carbon atoms, such as diamyl benzoic acid, hexadecyl-benzoic acid, wax benzoic acid, etc.; and naphthenic acids, such as those derived from petroleum.

(b) Phenolic acids, such as alkyl-substituted phenols, naphthols, resorcinols, catechols, hydroquinols, pyrogallol, etc., wherein the alkyl portion contains at least about 10 carbon atoms. As non-limiting examples of such acids, there may be mentioned diamyl phenol, wax phenol, dinonyl catechol, hexadecyl hydroquinone, wax pyrogallol, etc.

(c) Organo-substituted phosphorus-containing acids, i.e., partial esters of phosphorus acids, such as alkyl-, alkaryl- and aralkyl-substituted phosphoric, phosphonic and phosphinic acids. Non-limiting examples of such acids are dodecyl phenyl phosphoric acid, octadecyl phosphonic acid and diamyl phosphinic acid.

(d) Organo-substituted sulfur-containing acids, i.e., partial esters of sulfonic acids, such as alkyl-, alkaryl- and aralkyl-substituted sulfonic acids and alkyl sulfuric acids. Examples of such acids are dodecyl phenyl sulfonic acid, wax benzene sulfonic acid, petroleum sulfonic acid and octadecyl sulfuric acid.

(e) Organo-substituted phosphorus- and sulfur-containing acids, i.e., partial esters of phosphorus- and sulfur-containing acids, such as alkyl-, alkaryl- and aralkyl-substituted thiophosphoric, thiophosphonic and thiophosphinic acids. Examples of these types of acids are the following: wax phenyl dithiophosphoric acid, didodecyl thiophosphonic acid and dihexadecyl phosphinic acid.

#### THE METAL ALCOHOLATE REACTANT

The metal alcoholates which have been found to form alkoxy complex metal salts with the aforesaid acids are the alcoholates of the metals of Groups I, II, III and IV of Mendeleeff's Periodic Table of the Elements. Thus, the alcoholates of potassium, calcium, barium, strontium, zinc, magnesium, aluminum and tin have been used successfully. The alcohols from which the metal alcoholates may be derived are monohydroxy alcohols, preferably the

aliphatic alcohols having from 1 up to about 20 carbon atoms. Suitable metal alcoholates are, for example, sodium methylate, calcium methylate, barium methylate, magnesium methylate, aluminum isopropylate, calcium butylate, potassium caprylate, barium decylate, calcium dodecylate, magnesium tetradecylate, zinc hexadecylate and magnesium octadecylate.

In order to fully illustrate the nature and manner of preparation of our complex metal alkoxy salts and their ability as additives for fuels and lubricating oils, the following examples and test results are presented.

#### Example 1.—Complex magnesium methoxy salt of tall oil acid containing two equivalents of magnesium

Three hundred grams of "Facoil CB," a refined tall oil acid obtained from National Southern Products Corporation, having an acid number of about 165, and analyzing about 45.4% rosin acids and about 47.8% fatty acids, was blended with 600 grams of a straight run kerosene of approximately 350° F. to 500° F. boiling range. The kerosene blend of tall oil was added to 21.5 grams of magnesium (two equivalents based on acid number of "Facoil CB") in the form of a slurry of magnesium methylate (prepared from metallic magnesium and methanol) in methanol. The reaction mixture was heated with stirring to about 120-125° C. over a period of 4 to 5 hours, in which time all the methanol was removed leaving a clear solution of the complex methoxy magnesium salt of "Facoil CB" in kerosene. The final product was filtered through "Hi-Flo" (a diatomaceous clay filter-aid) to remove any traces of unreacted material. The product analyzed 2.4% magnesium in the kerosene blend which approximates theoretical magnesium for a complex methoxy magnesium salt of "Facoil CB" containing two equivalents of magnesium.

#### Example 2.—Complex magnesium methoxy salt of tall oil acid containing three equivalents of magnesium

Two hundred grams of "Facoil CB" (see Example 1) was blended with 400 grams of a solvent-refined mineral oil having a Saybolt viscosity of 35 seconds at 210° F. and added to 21.5 grams of magnesium (three equivalents based on the acid number of the "Facoil CB") in the form of a slurry of magnesium methylate in methanol. The temperature of the mixture was raised to about 120° C. to 125° C. over a period of 5 to 6 hours followed by filtration through "Hi-Flo" clay. The oil blend of the product analyzed 2.4% magnesium which was the theoretical magnesium content of a complex methoxy magnesium salt of "Facoil CB" containing three equivalents of magnesium.

#### Example 3.—Complex magnesium methoxy salt of tall oil acid containing four equivalents of magnesium

Two hundred grams of "Facoil CB" (see Example 1) was blended with 600 grams of kerosene and added to 28 grams of magnesium (four equivalents based on acid number of "Facoil CB") in the form of a slurry of magnesium methylate (see Example 1) in methanol. The temperature of the mixture was raised to about 120° C. to 125° C. over a period of 5 to 6 hours. Filtration through a layer of "Hi-Flo" clay yielded the final product which analyzed 3.5% magnesium in the kerosene blend. This analysis approximates the theoretical magnesium content of a complex methoxy magnesium salt of "Facoil CB" containing four equivalents of magnesium.

#### Example 4.—Complex magnesium methoxy salt of tall oil acid containing six equivalents of magnesium

One hundred grams of "Facoil CB" (see Example 1) was blended with 400 grams of kerosene and added to 21.5 grams of magnesium (six equivalents based on acid number of the "Facoil CB") in the form of a slurry of magnesium methylate (see Example 1) in methanol. The temperature of the mixture was raised to about 120°

C. to 125° C. over a period of 6 to 7 hours. Filtration through "Hi-Flo" clay yielded the final product analyzing 3.98% magnesium in the kerosene blend, which approximates theoretical magnesium content for a complex methoxy magnesium salt of "Facoil CB" containing six equivalents of magnesium.

*Example 5.—Complex calcium methoxy salt of tall oil acid containing two equivalents of calcium*

Two hundred grams of "Facoil CB" (see Example 1) was blended with 800 grams of kerosene and added to 23.6 grams of calcium (two equivalents based on acid number of the "Facoil CB") in the form of a slurry of calcium methylate (prepared from metallic calcium and methanol) in methanol. The temperature of the mixture was raised to about 120° C. to 125° C. over a period of 4 to 5 hours. Filtration through "Hi-Flo" clay yielded the final product analyzing 2.0% calcium in the kerosene blend, which approximates theoretical calcium content for a complex methoxy calcium salt of "Facoil CB" containing two equivalents of calcium.

*Example 6.—Complex magnesium methoxy salt of tall oil acid containing four equivalents of magnesium*

A complex methoxy magnesium salt of "Facoil CB" containing four equivalents of magnesium (similar to that of Example 3) was prepared by the following alternative procedure:

Fifty-four grams of sodium (four equivalents based on acid number of the "Facoil CB" in the form of sodium methylate was added to a methanol solution of 113 grams of anhydrous magnesium chloride (four equivalents based on acid number of "Facoil CB") and the mixture refluxed for 2 hours forming a methanol slurry of magnesium methylate and sodium chloride. To this slurry was added a blend of 200 grams of "Facoil CB" and 600 grams of kerosene. The reaction mixture was heated with stirring to about 120° C. to 125° C. over a period of 4 to 6 hours. Filtration through "Hi-Flo" clay yielded the final product analyzing 3.4% magnesium in the kerosene blend which approximates the theoretical magnesium content of Example 3.

*Example 7.—Complex zinc methoxy salt of naphthenic acid containing two equivalents of zinc*

Thirty-three grams of sodium (two equivalents based on acid number of the naphthenic acid) in the form of sodium methylate was added to a methanol solution of 98 grams of anhydrous zinc chloride (two equivalents based on the acid number of the naphthenic acid) and the mixture refluxed for two hours forming a methanol slurry of zinc methylate and sodium chloride. To this slurry was added a blend of 200 grams of naphthenic acid with an acid number of about 200 and 400 grams of a solvent refined mineral oil having a Saybolt viscosity of 35 seconds at 210° F. The reaction mixture was heated with stirring to about 125° C. over a period of about 5 hours and filtered through "Hi-Flo" clay. The oil blend of the product analyzed 7.3% zinc which was the theoretical zinc content for a complex methoxy zinc salt of naphthenic acid containing two equivalents of zinc.

*Example 8.—Complex zinc methoxy salt of naphthenic acid containing three equivalents of zinc*

A methanol solution of 147 grams of anhydrous zinc chloride (three equivalents based on acid number of naphthenic acid) was added to 49.5 grams of sodium (three equivalents based on acid number of naphthenic acid) in the form of sodium methylate and the mixture refluxed for two hours forming a methanol slurry of zinc methylate and sodium chloride. To this slurry was added a blend of 200 grams of naphthenic acid with an acid number of 200 and 400 grams of a solvent re-

fined mineral oil having a Saybolt viscosity of 35 seconds at 210° F. The reaction mixture was heated to about 125° C. over a period of about 5 hours and filtered through "Hi-Flo" clay. The oil blend of the product analyzed 10.4% zinc which was the theoretical zinc content for a complex methoxy zinc salt of naphthenic acid containing three equivalents of zinc.

*Example 9.—Complex zinc methoxy salt of naphthenic acid containing four equivalents of zinc*

Utilizing the procedure of Example 6, a complex zinc methoxy salt of naphthenic acid (M. W. 300) containing four equivalents of zinc was prepared as follows: Sixty-six grams of sodium (four equivalents based on acid number of the naphthenic acid) in the form of sodium methylate was added to a methanol solution of 196 grams of anhydrous zinc chloride (four equivalents based on acid number of the naphthenic acid) and the mixture refluxed for 2 hours forming a methanol slurry of zinc methylate and sodium chloride. To this slurry was added a blend of 200 grams of petroleum derived naphthenic acid, having an acid number of about 200, and 600 grams of kerosene. The reaction mixture was heated with stirring to about 120° C. to 125° C. over a period of about 5 hours, then filtered through "Hi-Flo" clay. The kerosene blend of the product analyzed 10.6% zinc which approximates the theoretical zinc content of a complex methoxy zinc salt of naphthenic acid containing four equivalents of zinc.

*Example 10.—Complex aluminum isopropoxy salt of naphthenic acid containing three equivalents of aluminum*

Seventy-three grams of aluminum isopropoxide (three equivalents based on acid number of the naphthenic acid) was dissolved in 400 grams of xylene by warming. The solution was added to 100 grams of naphthenic acid (see Example 9) and the mixture was heated with stirring to about 125° C. over a period of about 5 hours. The reaction mixture became clear and homogeneous at this point but was filtered through "Hi-Flo" clay as a precautionary measure to give the final product. The xylene blend of complex isopropoxy aluminum salt of naphthenic acid analyzed for 1.7% aluminum which was almost theoretical aluminum content for three equivalents of aluminum per equivalent of acid.

*Example 11.—Complex barium methoxy salt of naphthenic acid containing two equivalents of barium*

One hundred grams of naphthenic acid (see Example 9) was blended with 300 grams of kerosene and added to 50 grams of barium (two equivalents based on acid number of the naphthenic acid) in the form of a barium methylate solution (prepared from barium oxide and methanol) in methanol. The reaction mixture was heated to about 125° C. over a period of about 5 hours, then filtered through a layer of "Hi-Flo" clay. The barium analysis of the kerosene blend was 10.1% barium which approximates the theoretical barium content of a complex methoxy barium salt of naphthenic acid containing two equivalents of barium.

*Example 12.—Complex magnesium methoxy salt of naphthenic acid containing two equivalents of magnesium*

Two hundred grams of naphthenic acid (acid number=200) was blended with 400 grams of oil and reacted with 17.5 grams of magnesium (two equivalents based on acid number of naphthenic acid) using the procedure described in Example 1. The oil blend of the product analyzed 2.0% magnesium which was the theoretical magnesium content for a complex methoxy magnesium salt of naphthenic acid containing two equivalents of magnesium.

*Example 13.—Complex magnesium methoxy salt of naphthenic acid containing three equivalents of magnesium*

Two hundred grams of naphthenic acid (acid number =200) was blended with 600 grams of oil and reacted with 26.0 grams of magnesium (three equivalents based on acid number of naphthenic acid) using the procedure described in Example 1. The oil blend of the product analyzed 2.5% magnesium which was the theoretical magnesium content for a complex methoxy magnesium salt of naphthenic acid containing three equivalents of magnesium.

*Example 14.—Complex magnesium methoxy salt of wax phenol (3—14) containing two equivalents of magnesium*

One hundred grams of a wax alkylated phenol (wax phenol 3—14) was blended with 200 grams of kerosene and added to 3.1 grams of magnesium (two equivalents based on phenol content of wax phenol [3—14]) in the form of a slurry of magnesium methylate in methanol. The reaction mixture was heated with stirring to about 150° C. over a period of about 4 to 5 hours and filtered through "Hi-Flo" clay. The kerosene blend of the final product analyzed 0.95% magnesium which is almost theoretical magnesium content for a complex methoxy magnesium salt of wax phenol (3—14) containing two equivalents of magnesium.

The wax phenol (3—14) utilized in this example was prepared as follows:

A paraffin wax melting at approximately 120° F. and predominantly comprised of hydrocarbons, having at least 20 and an average of about 24 carbon atoms in their molecules, is melted and heated to about 200° F., after which chlorine is bubbled therethrough until the wax has absorbed about 14%, by weight, of chlorine. A sufficient quantity of this chlorinated wax to provide 3 atomic proportions of chlorine is then heated to a temperature varying from just above its melting point to not over 150° F. One mol of phenol ( $C_6H_5OH$ ) is then mixed with the chlorowax. The mixture is then heated to about 150° F. and a quantity of anhydrous aluminum chloride, corresponding to about 3% of the weight of the chlorowax in the mixture, is slowly added with active stirring. The rate of addition of the aluminum chloride should be sufficiently slow to avoid violent foaming and during the addition the temperature should be held at about 150° F. After the aluminum chloride has been added, the temperature of the mixture may be increased slowly over a period of from 15 to 25 minutes to a temperature of about 250° F. and then should be more slowly increased to about 350° F. To control the evolution of HCl gas, the temperature of the mixture is preferably raised from 250° F. to 350° F. at a rate of approximately one degree per minute, the whole heating operation occupying approximately two hours from the time of adding the aluminum chloride. If the emission of HCl gas has not ceased when the final temperature is reached, the mixture may be held at 350° F. for a short time to allow completion of the reaction. However, to avoid possible cracking of the wax, the mixture should not be heated appreciably above 350° F., nor should it be held at that temperature for any extended length of time.

It is important that all unreacted, or non-alkylated, phenol remaining in the reaction mixture, as well as aluminum chloride, be removed. This can be conveniently effected by washing the product several times with a mixture of water and an alcohol, such as butanol, preferably at elevated temperature, say 175° F. The product may then be treated with steam. This latter step will insure complete removal of the unreacted material and also dry the product.

It will be understood that a wax-substituted phenol prepared according to the above procedure in which a quantity of chlorowax containing 3 atomic proportions of chlorine and having a chlorine content of 14% is re-

acted with one mol of phenol is designated as "wax phenol (3—14)." Similarly, "wax phenol (3—10)" and "wax phenol (1—10)" may also be prepared by the reaction of sufficient amounts of chlorinated wax, containing 10%, by weight, of chlorine, to provide 3 atomic proportions and 1 atomic proportion of chlorine per mol of phenol, respectively, in the reaction and are useful in the invention. In general, the amount of chlorowax, containing from about 10% to 18%, by weight, of chlorine, used in the reaction is sufficient to supply between 1 and 4 atomic proportions of chlorine per mol of phenol.

*Example 15.—Complex sodium butoxy salt of wax phenol (3—14) containing two equivalents of sodium*

Two hundred grams of wax phenol (3—14) (see Example 14) was blended with 600 grams of kerosene and added to 11.5 grams of sodium (two equivalents based on the phenol content of the wax phenol [3—14]) in the form of a butanol solution of sodium butylate. The reaction mixture was heated with stirring to about 150° C. to 160° C. over a period of about 5 hours and filtered through "Hi-Flo" clay. The kerosene blend of the final product analyzed 1.2% sodium which was the theoretical sodium content for a complex butoxy sodium salt of wax phenol (3—14) containing two equivalents of sodium.

*Example 16.—Complex magnesium methoxy salt of wax-beta-naphthol (3—14) containing two equivalents of magnesium*

One hundred grams of wax alkylated beta-naphthol (3—14), prepared by the method given in Example 14 for the preparation of wax phenol (3—14), but using beta-naphthol in place of phenol, was blended with 200 grams of a solvent refined oil having a Saybolt viscosity of 35 seconds at 210° F. and added to 3.1 grams of magnesium (two equivalents based on the beta-naphthol content of wax-beta-naphthol [3—14]) in the form of a slurry of magnesium methylate in methanol. The reaction mixture was heated with stirring to about 150° C. over a period of about 5 hours and filtered through "Hi-Flo" clay. The oil blend of the final product analyzed 0.95% magnesium which approximates the theoretical magnesium content of a complex magnesium salt of wax-beta-naphthol (3—14) containing two equivalents of magnesium.

*Example 17.—Complex barium methoxy salt of petroleum sulfonic acid containing two equivalents of barium*

Four hundred and twenty-six grams of an aromatic petroleum stock sulfonic acid having an acid number of 32.8 was blended with 426 grams of a solvent refined mineral oil having a Saybolt viscosity of 35 seconds at 210° F. and the blend added to 34.2 grams of barium (two equivalents based on the acid number of the petroleum sulfonic acid) in the form of a barium methylate solution in methanol. The reaction mixture was heated with stirring to about 160° C. over a period of about 5 hours and filtered through "Hi-Flo" clay. The oil blend of the final product analyzed 3.7% barium which was the theoretical barium content for a complex methoxy barium salt of the particular petroleum sulfonic acid containing two equivalents of barium.

*Example 18.—Complex barium methoxy salt of wax benzene (2—12) sulfonic acid containing two equivalents of barium*

One hundred and eighty-two grams of a wax-alkylated benzene sulfonic acid having an acid number of 77.0 was blended with 364 grams of a solvent refined mineral oil having a Saybolt viscosity of 35 seconds at 210° F. and added to 34.2 grams of barium (two equivalents based on the acid number of the sulfonic acid) in the form of a barium methylate solution in methanol. The reaction mixture was heated with stirring to about 150° C. over a period of about 5 hours and filtered through "Hi-Flo"

clay. The oil blend of the product analyzed 5.34% barium which was the theoretical barium content for a complex methoxy barium salt of the wax-alkylated benzene sulfonic acid containing two equivalents of barium.

The wax benzene sulfonic acid utilized in this example was prepared as follows:

A paraffin wax having an average of 24 carbon atoms per molecule and a melting point of 126° F. was chlorinated at a temperature of about 100° C. with chlorine gas until the weight of the wax had increased about 12%. The chlorowax thus obtained was then blown with nitrogen to remove any occluded chloride and hydrogen chloride.

A 1000-gram portion of the chlorowax was then mixed with 500 grams of benzene in a 3-necked flask equipped with a stirrer, reflux condenser and a thermometer. The mixture was heated to a temperature of 60° C. Aluminum chloride was then added slowly over a period of two hours. The addition of aluminum chloride was accompanied by a vigorous evolution of hydrogen chloride. The temperature was then raised to a temperature of 80° C. and held there for one hour. The excess benzene was then removed by inverting the reflux condenser and heating to a temperature of 116° C. Two hundred milliliters of benzene were thus recovered. The mixture was cooled to a temperature of 60° C. and then another 1000 grams of chlorowax were added slowly. After completing the addition of this chlorowax, the temperature was raised to 100° C. and held there for one hour. The product was allowed to stand overnight at a temperature of about 60° C., and then was separated from the sludge by decantation and filtered by suction through clay.

Seventeen hundred and thirty-eight grams of wax benzene thus obtained were placed in a 3-necked flask equipped with a stirrer and a thermometer and heated to a temperature of 40° C. Eight hundred and sixty-nine grams of oleum (15% SO<sub>3</sub>) were added slowly to the wax benzene from a dropping funnel at a rate regulated to maintain the temperature below 50° C. The addition of oleum consumed about 3 hours. The mixture was then stirred for an additional hour to ensure complete reaction. The mixture was then poured into 1000 milliliters of water and subsequently 1810 grams of mineral oil were added to the mixture. The mixture thus obtained was stirred thoroughly and then allowed to stand until the water separated into a layer. The water layer was then drained off. The product thus obtained was approximately a 50% blend of wax benzene sulfonic acid in mineral oil and had a neutralization number of 40.7.

It will be understood that a wax benzene prepared according to the foregoing procedure in which a quantity of chlorowax containing 2 atomic proportions of chlorine and having a chlorine content of 12% is reacted with 1 mol of benzene is designated "wax benzene (2-12)." Similarly, "wax benzene (3-10)" and "wax benzene (1-10)" may also be prepared by the reaction of sufficient amounts of chlorinated wax, containing 10% by weight of chlorine, to provide 3 atomic proportions and 1 atomic proportion of chlorine per mol of benzene, respectively, in the reaction and are useful in the invention. In general, the amount of chlorowax containing from about 10% to about 18% by weight of chlorine used in the reaction is sufficient to supply between 1 and 4 atomic proportions of chlorine per mol of benzene used.

*Example 19.—Complex calcium methoxy salt of wax benzene (2-12) sulfonic acid containing two equivalents of calcium*

One hundred grams of a wax alkylated benzene sulfonic acid (2-12), prepared as described in Example 18, having an acid number of 84.0 was blended with 200 grams of a solvent refined mineral oil having a Saybolt viscosity of 35 seconds at 210° F. and added to 6.0 grams of calcium (two equivalents based on the acid number of the sulfonic acid) in the form of a slurry of calcium methylate in

methanol. The reaction mixture was heated with stirring to about 150° C. over a period of about 5 hours and filtered through "Hi-Flo" clay. The oil blend of the product analyzed 2.1% calcium which was the theoretical calcium content for a complex methoxy calcium salt of the wax-alkylated benzene sulfonic acid containing two equivalents of calcium.

*Example 20.—Complex sodium methoxy salt of wax benzene (2-12) sulfonic acid containing two equivalents of sodium*

Two hundred and twenty grams of a wax-alkylated benzene sulfonic acid (2-12), prepared as in Example 18, having an acid number of 80.0 was blended with 440 grams of a solvent refined mineral oil having a Saybolt viscosity of 35 seconds at 210° F. and added to 14.5 grams of sodium (two equivalents based on the acid number of the sulfonic acid) in the form of a sodium methylate solution in methanol. The reaction mixture was heated with stirring to about 150° C. over a period of about 5 hours and filtered through "Hi-Flo" clay. The oil blend of the product analyzed 2.1% sodium which was the theoretical sodium content for a complex methoxy sodium salt of the wax alkylated benzene sulfonic acid containing two equivalents of sodium.

*Example 21.—Complex magnesium methoxy salt of wax benzene (2-12) sulfonic acid containing two equivalents of magnesium*

Two hundred grams of a wax-alkylated benzene sulfonic acid (2-12), prepared as in Example 18, having an acid number of 77.0 was blended with 400 grams of a solvent refined mineral oil having a Saybolt viscosity of 35 seconds at 210° F. and added to 6.6 grams of magnesium (two equivalents based on the acid number of the sulfonic acid) in the form of a slurry of magnesium methylate in methanol. The reaction mixture was heated with stirring to about 150° C. over a period of about 5 hours and filtered through "Hi-Flo" clay. The oil blend of the product analyzed 0.95% magnesium which approximates the theoretical magnesium content of a complex methoxy magnesium salt of the wax alkylated benzene sulfonic acid containing two equivalents of magnesium.

*Example 22.—Complex potassium butoxy salt of wax benzene (2-12) sulfonic acid containing two equivalents of potassium*

Two hundred and fifty-three grams of a wax-alkylated benzene sulfonic acid (2-12), prepared as in Example 18, having an acid number of 88.0 was blended with 506 grams of a solvent refined mineral oil having a Saybolt viscosity of 35 seconds at 210° F. and added to 44.6 grams of potassium hydroxide (two equivalents based on the acid number of the sulfonic acid) in the form of a butanol solution of the potassium hydroxide. The reaction mixture was heated with stirring to about 175° C. over a period of about 5 hours and filtered through "Hi-Flo" clay. The oil blend of the product analyzed 4.0% potassium which was the theoretical potassium content for a complex butoxy potassium salt of the wax-alkylated benzene sulfonic acid containing two equivalents of potassium.

*Example 23.—Complex magnesium methoxy salt of dodecylphenyl phosphoric acid containing two equivalents of magnesium*

One hundred grams of a dodecylphenyl phosphoric acid having an acid number of 162 was blended with 200 grams of a solvent refined mineral oil having a Saybolt viscosity of 35 seconds at 210° F. and added to 7.0 grams of magnesium (two equivalents based on the acid number of the phosphoric acid) in the form of a slurry of magnesium methylate in methanol. The reaction mixture was heated with stirring to about 150° C. over a period of about 5 hours and filtered through "Hi-Flo" clay.

The oil blend of the product analyzed 2.3% magnesium which was the theoretical magnesium content for a complex methoxy magnesium salt of the dodecylphenyl phosphoric acid containing two equivalents of magnesium.

The dodecylphenyl phosphoric acid used in this example was prepared as follows: Two thousand grams of a dodecylphenol was stirred with 321 grams of phosphorus pentoxide and heated to 150° C. The reaction mixture was stirred at 150° C. for 3 hours and then filtered through "Hi-Flo" clay to give the finished dodecylphenyl phosphoric acid.

*Example 24.—Complex magnesium methoxy salt of wax phenyl dithiophosphoric acid containing three equivalents of magnesium*

Two hundred grams of a wax phenyl dithiophosphoric acid having an acid number of 46 was blended with 400 grams of a solvent refined mineral oil having a Saybolt viscosity of 35 seconds at 210° F. and added to 6.0 grams of magnesium (three equivalents based on the acid number of the dithiophosphoric acid) in the form of a slurry of magnesium methylate in methanol. The reaction mixture was heated with stirring to about 150° C. over a period of about 5 hours and filtered through "Hi-Flo" clay. The oil blend of the product analyzed 0.9% magnesium which approximates the theoretical magnesium content of a complex methoxy magnesium salt of the wax phenyl dithiophosphoric acid containing three equivalents of magnesium.

The wax phenyl dithiophosphoric acid used in this example was prepared as follows. An oil blend containing 387 grams of wax phenol (4—18) and 77.4 grams of the mineral oil described in Example 24 was stirred with 55.5 grams of phosphorus pentasulfide. The temperature of the reaction mixture was raised to 170° C. and held there for 5 hours. The final product was a wax phenyl dithiophosphoric acid having an acid number of about 46.

#### EVALUATION OF PRODUCTS

Test results showing the utility of the complex metal alkoxy salts as stabilizing agents for fuels and oils are presented in Tables I to IV. The effectiveness of the salts as color stabilizers and sludge inhibitors in a typical fuel oil in storage is shown by the data in Table I. It will be noted that sedimentation was substantially inhibited by the incorporation of the complex salt products in the oil and particularly so by the salts containing the higher equivalents of metal. The fuel used was comprised of 70% catalytically cracked fuel and 30% straight run fuel and had a boiling range of 350° F. to 650° F.

The test used was that described in A. S. T. M. Standards on Petroleum Products and Lubricants, September 1945, Test No. D665—44T. In this test, 350 cc. of test oil are placed in a tall form (127 x 70 mm.) beaker and a cylindrical polished steel specimen is suspended and soaked in the oil under test at 140° F. for 30 minutes. Thirty cc. of distilled water are added and the mixture is stirred at 1000 R. P. M. After 48 hours, the steel specimen is removed and examined for evidence of rust thereon. The specifications require the complete absence of rust, even pin points of rust, and the absence of dark stain. The fuel used was the same as that used in the fuel storage tests of Table I. The products have also been tested as anti-rust agents in gasoline and lubricating oil and found to give good results.

TABLE II.—A. S. T. M. RUST TEST

|    | Compound Added                                                   | Metal Equivalents | Concn., p. p. m. | Result |
|----|------------------------------------------------------------------|-------------------|------------------|--------|
| 20 | None                                                             |                   | 0                | Fail.  |
|    | Complex Magnesium Methoxy Salt of "Facoil CB" (Ex. 1).           | 2                 | 100              | Pass.  |
| 25 | Complex Magnesium Methoxy Salt of "Facoil CB" (Ex. 3).           | 4                 | 100              | Pass.  |
|    | Complex Sodium Methoxy Salt of Wax Phenol (Ex. 15).              | 2                 | 100              | Pass.  |
|    | Complex Magnesium Methoxy Salt of Naphthenic Acid.               | 4                 | 100              | Pass.  |
|    | Complex Barium Methoxy Salt of Petroleum Sulfonic Acid (Ex. 17). | 2                 | 100              | Pass.  |

The ability of the compounds of the invention as lubricating oil detergents was tested by the Lauson D-4A Detergency Test. This test determines the effectiveness of the lubricating oil in preventing fouling as measured by the cleanliness of rings, lands, ring grooves and piston-skirts. A single cylinder, 4-cycle, liquid cooled Lauson engine with splash lubrication and having a copper-lead bearing is used. The operating conditions are as follows:

Oil temperature 225° F.  
Jacket temperature 275° F.  
Speed 1825 R. P. M.  
Brake load 1.6 H. P.  
One-half throttle.  
13-1 air-fuel ratio.  
Oil added every 20 hours (one-gallon sample used).

The fuel used is a controlled "Mobilgas Special" type blend gasoline (40% thermal, 30% catalytically cracked and 30% straight run, plus 2.5 cc. TEL/gal.). The duration of the test is 100 hours.

An SAE 20 solvent-refined Pennsylvania oil was used

TABLE I

| Compound Added                                                       | Metal Equivalents | Concn.,<br>Lb./1,000<br>Bbls. | Six Weeks' Storage @<br>100° F. |                     |
|----------------------------------------------------------------------|-------------------|-------------------------------|---------------------------------|---------------------|
|                                                                      |                   |                               | N. P. A.                        | Sediment,<br>Mg./l. |
| None                                                                 |                   | 0                             | 8                               | 110                 |
| Complex Magnesium Methoxy Salt of "Facoil CB" (Example 1).           | 2                 | 50                            | 8                               | 12                  |
| Complex Magnesium Methoxy Salt of "Facoil CB" (Example 3).           | 4                 | 50                            | D6                              | 9                   |
| Complex Magnesium Methoxy Salt of "Facoil CB" (Example 4).           | 6                 | 50                            | D6                              | 9                   |
| Complex Calcium Methoxy Salt of "Facoil CB" (Example 5).             | 2                 | 100                           | 8                               | 23                  |
| Complex Zinc Methoxy Salt of Naphthenic Acid (Example 7).            | 2                 | 50                            | L2½                             | 13                  |
| Complex Aluminum Isopropyl Salt of Naphthenic Acid (Example 10).     | 3                 | 50                            | 8                               | 42                  |
| Complex Barium Methoxy Salt of Naphthenic Acid (Example 11).         | 2                 | 50                            | 8                               | 15                  |
| Complex Magnesium Methoxy Salt of Wax Phenol (Example 14).           | 2                 | 50                            | 8                               | 29                  |
| Complex Sodium Methoxy Salt of Wax Phenol (Example 15).              | 2                 |                               | L3½                             | 27                  |
| Complex Barium Methoxy Salt of Petroleum Sulfonic Acid (Example 17). | 2                 | 100                           | L7                              | 24                  |

Table II shows the effectiveness of the compounds of the invention as anti-rust agents in a typical fuel oil.

as the reference oil and various oil blends of the reference oil and the compounds of the invention were

tested in the engine separately. At the end of each run, the piston of the engine was examined and rated for lacquer and sludge deposits, an E. C. (Engine Cleanliness) Rating of 100 indicating a perfectly clean piston and lower ratings indicating increasing amounts of deposits. The test results are presented in Table III.

TABLE III.—LAUSON D4 PISTON DETERGENCY TEST

| Compound Added                                                              | Metal equivalents | Concn., Wt. percent | E. C. Rating |
|-----------------------------------------------------------------------------|-------------------|---------------------|--------------|
| None                                                                        |                   | 0                   | 62           |
| Complex Magnesium Methoxy Salt of "Facoil CB" (Ex. 1)                       | 2                 | 1                   | 67           |
| Complex Magnesium Methoxy Salt of "Facoil CB" (Ex. 2)                       | 3                 | 1                   | 74           |
| Complex Zinc Methoxy Salt of Naphthenic Acid (Ex. 7)                        | 2                 | 2                   | 76           |
| Complex Magnesium Methoxy Salt of Naphthenic Acid (Ex. 12)                  | 2                 | 1                   | 79           |
| Complex Magnesium Methoxy Salt of Naphthenic Acid (Ex. 13)                  | 3                 | 1                   | 77           |
| Complex Magnesium Methoxy Salt of Naphthenic Acid                           | 4                 | 1                   | 88           |
| Complex Magnesium Methoxy Salt of Wax Phenol (Ex. 14)                       | 2                 | 1                   | 77           |
| Complex Magnesium Methoxy Salt of Wax-B-Naphthol (Ex. 16)                   | 2                 | 1                   | 76           |
| Complex Barium Methoxy Salt of Wax Benzene Sulfonic Acid (Ex. 18)           | 2                 | 1                   | 77           |
| Complex Calcium Methoxy Salt of Wax Benzene Sulfonic Acid (Ex. 19)          | 2                 | 1                   | 87           |
| Complex Sodium Methoxy Salt of Wax Benzene Sulfonic Acid (Ex. 20)           | 2                 | 1                   | 84           |
| Complex Magnesium Methoxy Salt of Wax Benzene Sulfonic Acid (Ex. 21)        | 2                 | 1                   | 86           |
| Complex Potassium Butoxy Salt of Wax Benzene Sulfonic Acid (Ex. 22)         | 2                 | 1                   | 80           |
| Complex Magnesium Methoxy Salt of Dodecyl Phenyl Phosphoric Acid (Ex. 23)   | 2                 | 1                   | 75           |
| Complex Magnesium Methoxy Salt of Wax Phenyl Dithiophosphoric Acid (Ex. 24) | 3                 | 1                   | 73           |

The anti-oxidant character of the compounds of the invention in lubricating oil was demonstrated by means of the Lauson OS2 Oxidation Stability Test. In this test a Lauson single cylinder, 4-cycle, liquid cooled engine with splash lubrication and a copper-lead bearing is operated at an oil temperature of 270° F. and a jacket temperature of 212° F. at 1825 R. P. M. at 1/2 throttle and a 13 to 1 air-fuel ratio for 100 hours, oil being added every 20 hours. The fuel used is a controlled "Mobilgas Special" type blend (40% thermal, 30% catalytically cracked and 30% straight run, plus 2.5 cc. TEL/gal.).

As in the D4-A test, an SAE 20 solvent-refined Pennsylvania oil was used as the reference oil and various oil blends of the reference oil and the compounds of the invention were tested in the engine separately. The copper-lead engine bearing was accurately weighed before and after each test run to determine the weight loss thereof resulting from corrosion. The results of the several tests are given in Table IV.

TABLE IV.—LAUSON OS2 OXIDATION STABILITY TEST

| Compound Added                                                              | Metal equivalents | Concn., Wt. percent | Bearing Wt. loss, mg. |
|-----------------------------------------------------------------------------|-------------------|---------------------|-----------------------|
| None                                                                        | 0                 | 0                   | 450                   |
| Complex Zinc Methoxy Salt of "Facoil CB" (Ex. 2)                            | 3                 | 0.75                | 82                    |
| Complex Zinc Methoxy Salt of Naphthenic Acid (Ex. 7)                        | 2                 | 1.0                 | 87                    |
| Complex Zinc Methoxy Salt of Naphthenic Acid (Ex. 8)                        | 3                 | 1.0                 | 61                    |
| Complex Zinc Methoxy Salt of Naphthenic Acid (Ex. 9)                        | 4                 | 0.5                 | 49                    |
| Complex Magnesium Methoxy Salt of Naphthenic Acid (Ex. 12)                  | 2                 | 1.0                 | 400                   |
| Complex Magnesium Methoxy Salt of Wax Phenyl Dithiophosphoric Acid (Ex. 24) | 3                 | 1.0                 | 130                   |

As demonstrated herein, the complex metal alkoxy salts of the invention, which are actually concentrated solutions containing from about 20% to about 50% of the complex metal salts, are effective improving agents for various petroleum oil fractions in concentrations ranging from as little as 0.01% (i. e., 100 parts per mil-

lion) as anti-rust agents in gasoline to from 0.5% to 2.0% as anti-oxidants and detergents in lubricating oils. However, the complex salts may be used in greater or lesser amounts than shown herein depending upon the particular oil fraction and the use for which it is intended. Thus, amounts of from as little as 0.001% up to about 10% comprise the effective concentration range.

The petroleum oil fractions may, of course, contain other addition agents along with the complex metal alkoxy salts of the invention, such as viscosity index improvers, extreme pressure agents, and pour point depressants, which it may be found desirable to add to said fraction.

Although the complex salts of this invention are intended primarily for use as additives for various petroleum oil fractions, they also find application in the manufacture of detergent soaps, dispersants, etc.

Although the principles of the invention have been illustrated herein by means of certain specific examples and tests, it is not intended that the scope of the invention be limited thereby, but only as indicated in the appended claims.

What is claimed is:

1. A mineral oil fraction containing a minor proportion, sufficient to stabilize said oil fraction against oxidation, of a complex alkoxy metal salt of an organic acid prepared by the method which comprises: reacting a hydrocarbon solution containing 1 equivalent proportion of a hydrocarbon-soluble organic acid having a molecular weight of from about 200 to about 1000 with from at least about 2 and up to about 6 equivalent proportions of a metal alcoholate derived from an aliphatic monohydroxy alcohol having from 1 up to about 20 carbon atoms and the metal constituent of which is selected from the metals of Groups I and II of Mendeleeff's Periodic Table of the Elements, at a temperature of from about 50° C. to about 200° C., the complex salt so produced having combined therein about 2 equivalents of metal per equivalent of organic acid where the metal of the metal alcoholate used in the reaction is a metal of group I and from about 3 to about 6 equivalents of metal where the metal of the metal alcoholate used in the reaction is a metal of group II.

2. A mineral lubricating oil containing a minor proportion, sufficient to stabilize said oil fraction against oxidation, of a complex alkoxy metal salt of an organic acid prepared by the method which comprises: reacting a hydrocarbon solution containing 1 equivalent proportion of a hydrocarbon-soluble organic acid having a molecular weight of from about 200 to about 1000 with from at least about 2 and up to about 6 equivalent proportions of a metal alcoholate derived from an aliphatic monohydroxy alcohol having from 1 up to about 20 carbon atoms and the metal constituent of which is selected from the metals of Groups I and II of Mendeleeff's Periodic Table of the Elements, at a temperature of from about 50° C. to about 200° C., the complex salt so produced having combined therein about 2 equivalents of metal per equivalent of organic acid where the metal of the metal alcoholate used in the reaction is a metal of group I and from about 3 to about 6 equivalents of metal where the metal of the metal alcoholate used in the reaction is a metal of group II.

3. A mineral lubricating oil containing a minor proportion, sufficient to stabilize said oil against oxidation, of a complex methoxy magnesium salt of a naphthenic acid prepared by the method which comprises: reacting an oil solution containing 1 equivalent proportion of an oil-soluble naphthenic acid having a molecular weight of from about 200 to about 1000 with from at least about 2 and up to about 6 equivalents of magnesium methylate, at a temperature of from about 50° C. to about 200° C., the complex salt so produced having combined therein from about 3 to about 6 equivalents of magnesium per equivalent of naphthenic acid.

4. A mineral lubricating oil containing a minor proportion, sufficient to stabilize said oil against oxidation, of a complex potassium methoxy salt of a wax-benzene sulfonic acid prepared by the method which comprises: reacting an oil solution containing 1 equivalent proportion of an oil-soluble wax-benzene sulfonic acid having a molecular weight of from about 200 to about 1000 with from at least about 2 and up to about 6 equivalent proportions of potassium methylate, at a temperature of from about 50° C. to about 200° C., the complex salt so produced having combined therein about 2 equivalents of potassium per equivalent of wax-benzene sulfonic acid.

5. A fuel oil containing a minor proportion, sufficient to stabilize said fuel oil against oxidation, of a complex alkoxy metal salt of an organic acid prepared by the method which comprises: reacting a hydrocarbon solution containing 1 equivalent proportion of a hydrocarbon-soluble organic acid having a molecular weight of from about 200 to about 1000 with from at least about 2 and up to about 6 equivalent proportions of a metal alcoholate derived from an aliphatic monohydroxy alcohol having from 1 up to about 20 carbon atoms and the metal constituent of which is selected from the metals of Groups I and II of Mendeleeff's Periodic Table of the Elements, at a temperature of from about 50° C. to about 200° C., the complex salt so produced having combined therein about 2 equivalents of metal per equivalent of organic acid where the metal of the metal alcoholate used in the reaction is a metal of group I and from about 3 to about 6 equivalents of metal where the metal of the metal alcoholate used in the reaction is a metal of group II.

6. A fuel oil containing a minor proportion, sufficient to stabilize said oil against oxidation, of a complex methoxy magnesium salt of a tall oil acid prepared by the method which comprises: reacting an oil solution containing 1 equivalent proportion of an oil-soluble tall oil acid having a molecular weight of from about 200 to about 1000 with from at least about 2 and up to about 6 equivalent proportions of magnesium methylate, at a temperature of from about 50° C. to about 200° C., the complex salt so produced having combined therein from about 3 to about 6 equivalents of magnesium per equivalent of tall oil acid.

7. A fuel oil containing a minor proportion, sufficient to stabilize said oil against oxidation, of a complex methoxy zinc salt of a naphthenic acid prepared by the method which comprises: reacting an oil solution containing 1 equivalent proportion of an oil-soluble naphthenic acid having a molecular weight of from about 200 to about 1000 with from at least about 2 and up to about 6 equivalent proportions of zinc methylate, at a temperature of from about 50° C. to about 200° C., the complex salt so produced having combined therein from about 3 to about 6 equivalents of zinc per equivalent of naphthenic acid.

8. A gasoline containing a minor proportion, sufficient to stabilize said gasoline against oxidation and inhibit the formation of rust therein, of a complex alkoxy metal salt of an organic acid and prepared by the method which comprises: reacting a hydrocarbon solution containing 1 equivalent proportion of a hydrocarbon-soluble organic acid having a molecular weight of from about 200 to about 1000 with from at least about 2 and up to about 6 equivalent proportions of a metal alcoholate derived from an aliphatic monohydroxy alcohol having from 1 up to about 20 carbon atoms and the metal constituent of which is selected from the metals of Group I and II of Mendeleeff's Periodic Table of the Elements, at a temperature of from about 50° C. to about 200° C., the complex salt so produced having combined therein about 2 equivalents of metal per equivalent of organic acid where the metal of the metal alcoholate used in the reaction is a metal of group I and from about 3 to about 6 equivalents of metal where the metal of the metal alcoholate used in the reaction is a metal of group II.

9. A gasoline containing a minor proportion, sufficient to stabilize said gasoline against oxidation and inhibit the formation of rust therein, of a complex methoxy magnesium salt of a tall oil acid prepared by the method which comprises: reacting an oil solution containing 1 equivalent proportion of an oil-soluble tall oil acid having a molecular weight of from about 200 to about 1000 with from at least about 2 and up to about 6 equivalent proportions of magnesium methylate, at a temperature of from about 50° C. to about 200° C., the complex salt so produced having combined therein from about 3 to about 6 equivalents of magnesium per equivalent of tall oil acid.

#### References Cited in the file of this patent

#### UNITED STATES PATENTS

|           |                      |                |
|-----------|----------------------|----------------|
| 2,113,243 | Scott et al. _____   | Apr. 5, 1938   |
| 2,225,197 | Stagner _____        | Dec. 17, 1940  |
| 2,469,041 | Jones _____          | May 3, 1949    |
| 2,528,803 | Unkefer _____        | Nov. 7, 1950   |
| 2,610,982 | Hutcheson _____      | Sept. 16, 1952 |
| 2,582,833 | Hunn _____           | Jan. 15, 1952  |
| 2,585,520 | Van Ess et al. _____ | Feb. 12, 1952  |

#### OTHER REFERENCES

Richters Organic Chemistry Vol. 11 3rd Ed., Nordemann Pub. Co., New York, N. Y., page 350 (1939).

Steele—Jr. American Chem. Soc.—Vol 44, page 1337 (1922).

Sloane—Jr. Oil and Colour Chem.—Vol. 5, pages 323-324 (1922).

Hasselstrom et al., Jr. American Chem. Soc. vol. 61 (1939) page 1229.

Fieser and Fieser, Org. Chem. 2nd Ed., D. C. Heath and Co., Boston, Mass., page 126.